

# UNITED STATES PATENT OFFICE.

JAMES G. KELLY, ALBERT L. PRINGLE, AND HOLMES HALL, OF SEDALIA, MISSOURI.

## BEARING METAL.

1,376,339.

Specification of Letters Patent. Patented Apr. 26, 1921.

No Drawing.

Application filed May 7, 1920. Serial No. 379,642.

To all whom it may concern:

Be it known that we, JAMES G. KELLY, ALBERT L. PRINGLE, and HOLMES HALL, citizens of the United States, residing at 5 the city of Sedalia, in the county of Pettis and State of Missouri, have invented certain new and useful Improvements in Bearing Metals, of which the following is a specification.

10 This invention consists of a bearing metal composed of zinc, aluminum, tin, and lead, which composition is very close-grained and very tough and has enduring qualities and when turned, bored, planed, filed, or scraped 15 will have a very smooth surface and withstand very heavy pressure at a very high rate of speed and which wears away very slowly.

The zinc and aluminum are used as a base 20 or to form the foundation of this bearing metal and to give hardness and toughness to the same. The zinc and aluminum are used in substantially equal proportions by weight or with a slightly greater percentage of one 25 than the other, and in practice we have used a slightly greater percentage of zinc than aluminum, although we have also obtained very satisfactory results by using a slightly greater percentage of aluminum 30 than zinc, and we have used the aluminum and zinc combined as constituting from 15 per cent. to 35 per cent. of the whole, the aluminum constituting from 5 per cent. to 15 per cent. of the whole and the zinc comprising from 10 per cent. to 20 per cent. of the whole.

The union of zinc and aluminum creates a new alloy which is tougher, smoother, and closer-grained and causes less friction than 40 either zinc or aluminum used separately.

The tin and lead are used to give the composition body and to overcome crystallization and to avoid brittleness and to form a composition that will have a smooth surface 45 and also to decrease and overcome friction. Sufficient quantities of tin and lead should be used so that, when combined with the zinc and aluminum, the composition will have a smooth surface and will not crystallize and will not heat by contact with the other metals as when used as a bearing metal in a journal-bearing composed of steel or other metals when run at a very high rate of speed, and yet the tin and 50 lead should not be used in such a proportion as will make the composition too soft,

but the aluminum and zinc should constitute a sufficient proportion of the whole to maintain hardness and toughness of the composition. The lead serves, also, as a 60 binder for the whole, which is a physical rather than a chemical union of ingredients. In our experiments we have used tin and lead in substantially the proportions by weight of two parts of tin to one part lead, 65 the tin and lead constituting from 65 per cent. to 85 per cent. of the whole.

Our preferred formula is 48 per cent. tin, 24 per cent. lead, 16 per cent. zinc, and 12 per cent. aluminum, but we have found that 70 this formula is susceptible to change and that in certain uses for bearing metal better results may be obtained by slightly changing our formula. When using our composition for bearings where the bearing surface 75 is small and where the machinery is run at an excessive rate of speed, the proportion of tin can be slightly increased and the proportions of lead and aluminum slightly decreased; and, on the other hand, when the 80 bearing surface is large and only a moderate speed is attained, the percentage of tin may be slightly decreased and the percentage of lead and aluminum and even the percentage of zinc may be increased and 85 equally good results obtained.

While the proportions above given are, as stated, susceptible to some variation without affecting or injuring the quality of this bearing metal, any substantial deviation from the 90 proportions given will impair the usefulness of the compound as a bearing metal. The bearing metal of the composition as above described is produced in the following manner:

First. Melt the aluminum and add the zinc to the melted aluminum, and as the zinc melts, keep stirring until all the zinc and aluminum are melted and thoroughly mixed; or melt the zinc and aluminum separately and pour the melted zinc and aluminum together and stir thoroughly until the 100 two are well mixed.

Second. When the aluminum and zinc are melted and thoroughly mixed together, skim 105 off the scum which forms on the top of this mixture with a strainer composed of some metal which will not melt from the heat of the melted zinc and aluminum.

Third. Add the lead and stir continuously 110 until the lead is melted and mixed with the aluminum and zinc.

Fourth. Add the tin and stir the mixture continuously until all the tin is melted and the mixture is thoroughly mixed and then pour into molds of the form desired.

5 A characteristic result of the materials combined in the proportions stated is that the resultant alloy is particularly adapted for use as a bearing metal. For example, the combination of the zinc and aluminum 10 gives that desired degree of hardness and toughness to the alloy best adapted for its use as a bearing metal when used in substantially equal proportions by weight, and this desired condition is disadvantageously affected when these proportions are changed. Again, the tin and lead, substantially in the proportions mentioned afford a smooth surface to avoid excessive friction, and also avoid brittleness. If the proportions named 15 are substantially departed from, experience has proven that crystallization and friction-heating will result. Hence the proportions named, both as to the relative part of each metal to the other and also to the whole, are 20 most effective for a bearing metal alloy, any substantial variation of such proportions resulting in a bearing metal having an undesirable characteristic for the particular use.

25 30 Having thus described this invention, we

hereby reserve the benefit of all changes in form, arrangement, order, or use of parts, as it is evident that many minor changes may be made therein without departing from the spirit of this invention or the scope of the 35 following claims:

We claim:

1. A bearing metal composed of tin, lead, zinc, and aluminum, substantially in the proportions of one part of aluminum, 40 slightly more than one part of zinc, two parts of lead and four parts of tin.

2. A bearing metal composed of tin, lead, zinc, and aluminum, the zinc and aluminum constituting from one-sixth to one-third of 45 the whole in the proportions of one part of aluminum, and a slightly greater proportion of zinc, the remainder of the composition being composed of tin and lead substantially in the proportions of two parts of tin to one 50 part of lead.

In testimony whereof we hereunto affix our signatures.

JAMES G. KELLY.  
ALBERT L. PRINGLE.  
HOLMES HALL.

Witnesses:

JOHN J. KELLY,  
W. D. O'BANNON.